

# UNITED STATES PATENT OFFICE.

BO MICHAËL STURE KALLING AND SVEN DAGOBERT DANIELI, OF TROLLHÄTTAN,  
SWEDEN, ASSIGNEES TO AKTIEBOLAGET FERROLEGERINGAR, OF STOCKHOLM,  
SWEDEN, A LIMITED COMPANY.

## METHOD FOR PRODUCING MANGANESE OR ALLOYS OF MANGANESE.

1,363,657.

Specification of Letters Patent. Patented Dec. 28, 1920.

No Drawing.

Application filed November 4, 1919. Serial No. 335,669.

*To all whom it may concern:*

Be it known that we, Bo MICHAËL STURE KALLING and SVEN DAGOBERT DANIELI, subjects of the King of Sweden, and residents of Trollhättan, in the Kingdom of Sweden, have invented certain new and useful Improvements in Methods for Producing Manganese or Alloys of Manganese, of which the following is a specification.

10 The present invention has for its object a process for manufacturing manganese or manganese-alloys with low content of carbon and silicon.

In accordance with the present invention, 15 the said products are obtained by subjecting a manganese alloy which is richer in silicon—preferably one which contains more than 20% manganese and more than 10% silicon—at a temperature higher than 100° C., to the action of substances which, under 20 certain conditions, will oxidize the silicon. As an oxidizing medium, free oxygen (air) is employed and, if necessary, substances which contain oxygen compound of manganese. 25 As silicate-forming ingredients, it is practicable to use such substances as contain manganese.

The following example will serve to make plain the invention.

30 As is known, in the manufacture of manganese and manganese alloys, with carbon as a reducing medium, the product actually obtained is a manganese carbid, or manganese carbid alloy, with a content of carbon which, 35 as a general rule, is not less than the equivalent of  $Mn_3C$ . Experiments have been made with a view of appreciably reducing the carbon content of the alloy in question, for example by treatment with manganese oxids, 40 but such experiments have not yielded the desired results.

It is also known that, if in the production of manganese and its alloys with carbon as a reducing medium, the process employed is 45 such that the silicon is reduced out together with the manganese, in the silico-manganese alloy obtained a larger or smaller part of the carbon will have been replaced by silicon.

A somewhat similar result is obtained if

the manganese alloy with a high content of 50 carbon is alloyed with a silicon alloy comparatively rich in silicon and consequently poor in carbon. In accordance with the present invention, such a silico-manganese alloy is treated at a suitable temperature 55 with silicon-oxidizing substances, especially such as contain lime and manganese oxids. A larger or smaller amount of the silicon is thereby oxidized and the alloy obtained as the final product—provided the reduction 60 process has taken place under such circumstances that the alloy or the oxidizing medium has not been allowed to get into touch with carboniferous substances—does not contain, strictly speaking, more carbon, at most, 65 than the quantity contained in the silico-manganese used in the charge. The oxidizing process is conveniently performed in an electric furnace of such construction that the electrodes are not in direct contact with the 70 reacting substances, for example an electric free burning arc-furnace.

The slag obtained in the oxidation of the silicon contains as a general rule, an appreciable content of manganese oxids, and may be 75 suitably used as a raw material for the manufacture of silico-manganese.

There is no objection to the manufacture of silico-manganese and the oxidation of its silicon taking place in the same furnace. In 80 this case, the silico-manganese alloy is first produced in the ordinary manner, whereupon any slag formed in the process is tapped off, and finally suitable oxidizing 85 mediums are added, whereby the silicon is oxidized.

The manufacture of the manganese alloy with low content of carbon can also be performed by the employment of two furnaces, in one of which the silico-manganese alloy 90 is produced in the usual manner, the said alloy being afterward transferred in molten condition into the other furnace, in order to be treated with silicon-oxidizing substances. In this case it may be found desirable to 95 heat the silicon-oxidizing substances prior to treatment to such a temperature that a reaction immediately sets in.

The oxidation of the silicon can also be carried out by thoroughly mixing an ordinary silico-manganese alloy in a solid state with the silicon-oxidizing and silicon-oxidizing substances, the mixture being afterward heated to a suitable temperature.

One manner of carrying out the improved process is to blow free oxygen, for example in the form of air, through a molten bath of silico-manganese in a Bessemer converter, of suitable construction, with basic, neutral or acid lining, with the addition, if necessary, of substances containing quick lime. In order to prevent an unnecessary increase of temperature, suitable quantities of substances containing oxides of manganese may eventually be added together with the lime-containing substance, and if a sufficient quantity of such substances is added to bring the manganese content of the slag to an adequate height, the oxidation of the manganese content of the silico-manganese will be prevented.

The manganese alloy with low content of silicon and carbon, manufactured in accordance with the present invention, as compared, for example with the ordinary ferro-manganese of commerce, is of greatest importance in the iron trade. In addition to the advantage that by the use of such an alloy, the necessity of appreciably increasing the content of carbon is avoided, as, for instance, when ferro-manganese is added to steel, there accrues, particularly, the advantage that the introduction into the steel itself of carbon monoxide, which otherwise arises by the oxidation of the carbon introduced with the ferro-manganese is obviated to the greatest possible extent, which is a matter of considerable importance for obtaining a material as free as possible from air blebs. The alloy in question is also extremely well suited for the production of steel with a high content of manganese and a relatively low content of carbon.

It will be obvious that if the oxidation of silicon in the manner above indicated is carried far enough, it will be possible to obtain, instead of a manganese alloy poor in carbon and silicon, a manganese which is practically free from silicon, so that the process can be adapted for the manufacture of manganese, just as well as for the manufacture of manganese alloys.

55 The process may also be performed in the following manner: As a basic material is used manganese oxide, which is reduced with carbon, at temperatures, and under charging conditions, suitable for the purpose, in such a way that the manganese silicid, *i. e.*, a silico-manganese alloy poor in carbon, is obtained, whereupon the latter intermediate product, in the manner above stated, *viz.*, without the material being allowed to come into contact with carbon, is oxidized in such

a way that a manganese alloy poor in carbon and silicon, or else manganese, is obtained.

The term "manganese alloy" in this description, and in the claims, is to be understood to mean not merely an alloy of manganese with heavy metals, but also as converging compounds of solutions of manganese with carbon, silicon, or similar substances, such as manganese carbide, manganese silicid, etc., as well as a solution of the said compounds in manganese or other metal.

Having thus described our invention, we declare, that what we claim is:

1. The process of manufacturing manganese alloys with low content of carbon and silicon, which consists in exposing a manganese alloy comparatively rich in silicon, at a temperature above the melting point of the alloy, to the oxidizing action of free oxygen.

2. The process of manufacturing manganese alloys with low content of carbon and silicon, which consists in exposing a manganese alloy containing more than 10 per cent of silicon, at a temperature above the melting point of the alloy, to the oxidizing action of free oxygen.

3. The process of manufacturing manganese alloys with low content of carbon and silicon, which consists in exposing a manganese alloy containing more than 10 per cent of silicon, at a temperature above the melting point of the alloy, to the oxidizing action of free oxygen simultaneously with substances containing oxygen compounds of manganese.

4. The process of manufacturing manganese alloys with low content of carbon and silicon, which consists in exposing a manganese alloy, comparatively rich in silicon, at a temperature above the melting point of the alloy, to the oxidizing action of free oxygen simultaneously with substances containing oxygen compounds of manganese together with other substances which are capable of dissolving silica or to form silicates therewith.

5. The process of manufacturing manganese alloys with low content of carbon and silicon, which consists in exposing a manganese alloy comparatively rich in silicon, at a temperature above the melting point of the alloy, to the oxidizing action of free oxygen simultaneously with substances containing oxygen compounds of manganese, and adding other substances capable of dissolving silica, no outer heat being supplied during the process.

6. The process of manufacturing manganese alloys with low content of carbon and silicon, which consists in exposing a manganese alloy containing more than 10 per cent of silicon at a temperature above the melting point of the alloy, to the oxidizing ac-

tion of free oxygen simultaneously with substances containing oxygen compounds of manganese, and adding other substances capable of dissolving silica, no outer heat being supplied during the process and the free oxygen, which is used as the silicon-oxidizing substance, being blown through the fluid silico-manganese alloy.

In witness whereof we have hereunto set our hands in presence of two witnesses.

BO MICHAËL STURE KALLING.  
SVEN DAGOBERT DANIELI.

Witnesses:

OSCAR SKARBERG,  
JOSEF JOHANSSON.